

# UNITED STATES PATENT OFFICE.

JOHN COLLINS, OF BROOKLYN, NEW YORK.

LINING GAS-GENERATORS, ACID-CHAMBERS, AND FOUNTAINS FOR MINERAL WATERS.

SPECIFICATION forming part of Letters Patent No. 231,540, dated August 24, 1880.

Application filed July 8, 1880. (No model.)

*To all whom it may concern:*

Be it known that I, JOHN COLLINS, of Brooklyn, in the county of Kings and State of New York, have invented a new and useful Improvement in Lining Gas-Generators, Acid-Chambers, and Fountains for Mineral Waters; and I do hereby declare that the following is a full, clear, and exact description of the same.

The object of this invention is to furnish a compound for lining gas-generators, acid-chambers, and fountains for mineral waters, the use of which will avoid the expense and labor involved in the ordinary method of lining said vessels.

15 The invention consists in a composition of matter to be used for lining gas-generators, acid-chambers, and fountains for mineral waters, consisting of asphaltum, benzine, and plumbago, and also in the method of lining 20 gas-generators, acid-chambers, and fountains for mineral waters, which consists in applying to their inner surfaces a compound of asphaltum, benzine, and plumbago, as will be herein-after fully described.

25 In carrying my invention into practical effect, I put any desired quantity of powdered asphaltum into a vessel suitable for heating, and pour over the asphaltum a sufficient quantity of deodorized benzine to reduce the said 30 asphaltum to a thick paste. The mixture is then heated until the asphaltum is fully dissolved, when powdered plumbago, in the proportion of pound to pound, is sprinkled upon the mixture. The heat is continued and the

compound thoroughly stirred for a few minutes, when it is ready for use. 35

The compound is applied with a brush to the inner surface of the gas-generators, acid-chambers, and fountains until the entire inner surface is thoroughly coated. When the coat 40 has become dry I smooth and polish it by rubbing with a cloth.

With this lining the gas and mineral waters will be prevented from coming in contact with and acting upon the surface of the vessels, 45 and at the same time the lining and the gas and mineral water will have no effect upon each other.

What I claim is—

1. The herein-described composition of matter to be used for lining gas-generators, acid-chambers, and fountains for mineral waters, consisting of asphaltum, benzine, and plumbago, in substantially the proportions specified. 50

2. The method of lining gas-generators, acid-chambers, and fountains for mineral waters, substantially as herein described, which consists in applying a compound of asphaltum, benzine, and plumbago to the inner surfaces 60 of the gas-generators, acid-chambers, and fountains, as set forth.

The above specification of my invention signed by me this 1st day of July, 1880.

JOHN COLLINS.

Witnesses:

AMOS W. HART,  
C. R. WRIGHT.